

No. 850,726.

PATENTED APR. 16, 1907.

J. H. BILLS.

APPARATUS FOR RECOVERING TIN AND SOLDER.

APPLICATION FILED JULY 11, 1906.

Fig. 1.



Fig. 2.



Fig. 3.



Inventor

J. H. Bills

Witnesses

Frank B. Hoffman  
Wm. Koerth

By Victor J. Evans

Attorney

# UNITED STATES PATENT OFFICE.

JOHN H. BILLS, OF LARAMIE, WYOMING, ASSIGNOR TO UNITED STATES TIN, SOLDER & IRON COMPANY, OF DENVER, COLORADO, A CORPORATION OF COLORADO

## APPARATUS FOR RECOVERING TIN AND SOLDER.

No. 850,726.

Specification of Letters Patent.

Patented April 16, 1907.

Application filed July 11, 1906. Serial No. 325,610.

*To all whom it may concern:*

Be it known that I, JOHN H. BILLS, a citizen of the United States, residing at Laramie, in the county of Albany and State of Wyoming, have invented new and useful Improvements in Apparatus for Recovering Tin and Solder, of which the following is a specification.

This invention relates to an improved apparatus and process for recovering tin and solder from scraps of tin-plate, old cans made of tin-plate, and like material which is frequently permitted to go to waste, the object of the invention being to recover and to save the tin and solder, which is comparatively valuable.

A further object of the invention is to provide an apparatus of simple and improved construction, whereby the process of recovering the tin and solder may be carried into operation efficiently and economically.

With these and other ends in view the invention consists in the improved construction and novel arrangement and combination of parts, which will be hereinafter fully described, and particularly pointed out in the claims.

In the accompanying drawings has been illustrated a simple and preferred form of an apparatus for carrying the invention into practical operation, it being, however, understood that no limitation is necessarily made to the precise structural details therein exhibited, but that changes, alterations, and modifications within the scope of the invention may be resorted to when desired.

In the drawings, Figure 1 is a longitudinal sectional view of an apparatus constructed in accordance with the principles of the invention. Fig. 2 is a vertical transverse sectional view of the same. Fig. 3 is a plan view showing the foraminous drum detached, together with the operating-shaft having the pulley and the fly-wheel.

Corresponding parts in the several figures are denoted by like characters of reference.

Upon a base 1 there are mounted uprights 2, constituting bearings for a shaft 3, having a driving-pulley 4 and a fly-wheel 5, the pulley 4 being used for the reception of power from any convenient source.

The shaft 3 carries a cylindrical drum 6,

which is preferably constructed of refractory metal, such as iron or copper, the cylindrical walls of said drum being provided with a large number of perforations 7. The drum 6 has been shown as provided with a hinged lid 8, forming a closure for an opening through which the drum may be charged with material to be operated upon and through which the scrap may afterward be removed.

Beneath the drum there has been constructed a furnace, of which 9 are the side walls and 10 the grate-bars. Any suitable fuel may be consumed in said furnace for the purpose of heating the drum and its contents.

I would have it understood that in place of a furnace such as has been conventionally shown in the drawings burners for the consumption of gas or vapor may be utilized within the scope of the invention. In any case, however, it is desirable that the upper ends of the furnace-walls be inclined in the direction of each other, as will be clearly seen in Fig. 2 of the drawings, a comparatively narrow slit or opening 11 being left between the upper edges of said furnace-walls.

Along the furnace-walls adjacent to the outer sides of the latter there are placed molds 12 for the reception of the tin and solder which is recovered by the use of the improved apparatus.

15 represents a hood or shield constituting the cover for the drum and furnace, the sides 16 of said hood being adapted to fit snugly upon the outer sides of the molds 12. When the hood or shield is placed in position, its upper portion is slightly spaced from the drum 6, as will be clearly seen in Figs. 1 and 2 of the drawings.

In the operation of this device the tin-plate from which the valuable metals are to be recovered and which, as stated, may be in the shape of old tin cans is deposited in the drum, beneath which a fire is ignited, after which the hood or shield is placed in position. When the drum becomes sufficiently heated to fuse the tin and solder upon the tin-plate contained therein, rotary motion at a considerable speed is imparted to the shaft carrying said drum, thus causing the molten tin and solder to be expelled by centrifugal ac-

tion through the apertures of the drum. When thus expelled, the molten metal will strike the hood or shield and the upper surfaces of the inclined portions of the side walls 9, whereby it will be guided into the molds 12, where it is permitted to accumulate, and subsequently to cool or harden into pigs or ingots. When the molds have been filled, they may be conveniently removed and empty ones substituted in place thereof. After the valuable metals have been recovered from the contents of the drum the scrap is removed from the latter, after which it may be recharged for a repetition of the operation.

It will be readily seen that the leading feature of the invention resides in the use of a foraminous drum or container which is supported for rotation in such a manner as to be capable of being rapidly rotated so as to cause the valuable metals, which have been reduced to a molten condition, to be expelled by centrifugal action through the perforations of said drum or container.

It is obvious that the old tin cans which constitute the material most frequently operated upon will become unsoldered, and the pieces of which they are composed will be agitated and shaken by the rotation of the drum, so that the molten tin or solder will be rapidly and thoroughly expelled. Hence by the present invention the valuable metals may be recovered and saved speedily with little manual labor and at a total expense

which is much below the value of the metals recovered by the operation.

The improved apparatus may be constructed and installed for operation at a small expense, and it may be successfully operated without having recourse to skilled labor.

What is claimed is—

1. An apparatus for recovering tin and solder from old tin-plate, including a foraminous container supported for rotation, means beneath the container for heating the latter and its contents, side walls beneath the container having their upper portions inclined in the direction of each other, molds disposed alongside of the side walls, and a hood arranged over the drum and the molds and fitting snugly against the latter.

2. In an apparatus of the class described, a foraminous drum supported for rotation, a furnace arranged beneath the drum and having side walls the upper portions of which are inclined in the direction of each other, receiving-molds disposed along the side walls and in contact therewith, and a hood or shield constituting a covering for the drum, the furnace and the molds, and fitting snugly against the latter.

In testimony whereof I affix my signature in presence of two witnesses.

JOHN H. BILLS.

Witnesses:

E. A. WILKINSON,  
W. A. STODDARD.